

# UNITED STATES PATENT OFFICE.

JOHN B. E. VENNER, OF MILWAUKEE, WISCONSIN.

## WOOD FILLER AND PRIMER COMPOUND AND THE METHOD OF PRODUCING THE SAME.

No. 893,287.

Specification of Letters Patent.

Patented July 14, 1908.

Application filed November 9, 1907. Serial No. 401,406.

*To all whom it may concern:*

Be it known that I, JOHN B. E. VENNER, a citizen of the United States, residing at Milwaukee, county of Milwaukee, and State of Wisconsin, have invented new and useful Improvements in Wood Filler and Primer Compound and the Method of Producing the Same, of which the following is a specification.

10 My composition consists of the following ingredients compounded in the proportions and manner hereinafter set forth, viz.— raw linseed oil 1 gallon, litharge  $\frac{1}{2}$  pound, sugar of lead  $\frac{1}{4}$  pound, benzin of sufficient quantity to reduce the same after having been boiled to the required consistency for application with the brush, and talc or mineral pulp 4 pounds. These ingredients are mingled together and treated as follows,— 20 the above named quantity of raw linseed oil is first boiled over a slow fire for a period of about 4 hours, when  $\frac{1}{2}$  pound of the litharge is added and thoroughly mixed. After the litharge has been thus added the oil is boiled for another hour when  $\frac{1}{4}$  pound of sugar of lead is added and thoroughly mixed. When the sugar of lead is thus added and mixed the compound is boiled slowly for an additional 25 4 or 5 hours longer until the same becomes of about the consistency of thick honey or balsam fir, so that when removed from the fire it is so elastic that it is capable of being drawn out and stretched like wax or gum. When the compound has been thus boiled and removed from the fire, benzin is applied until it is dissolved and liquefied to the consistency of varnish or paint so that it may be readily spread in the ordinary manner with a brush. When thus dissolved about 40 4 pounds of mineral pulp or talc is applied and thoroughly mixed therewith when the compound is ready for use.

I am aware that thin linseed oil has heretofore been thickened by commingling therewith solid substances until the same was of the proper consistency to be applied, with the present compound, however, the oil is thickened to the desired consistency to form the body of the filler by boiling until it is brought to the wax like condition described, when the benzin is added solely for the purpose of reducing it to the required consist-

ency for application. When thus thinned by the benzin it readily penetrates the surface of the wood, when the benzin quickly 55 evaporates leaving the oil upon and beneath the surface of the wood. The compound thus formed when applied to wood will impart an attractive tone and color and produce a smooth durable surface which is adapted to 60 not only preserve the wood but to give it a neat and finished appearance.

Having thus described my invention, I claim—

1. As a filler and primer, the herein described composition of matter consisting of linseed oil boiled to the consistency of thick honey, litharge, sugar of lead, talc, and benzin compounded together, boiled and treated substantially as described and for the purposes specified.

2. The herein described composition of matter to be used as filler or primer compounded in the following proportions,—linseed oil about 1 gallon boiled to the consistency of thick honey, litharge about  $\frac{1}{2}$  pound, sugar of lead about  $\frac{1}{4}$  pound, benzin of sufficient quantity to reduce the same for application, and talc about 4 pounds compounded together, boiled and treated substantially as described.

3. The method of manufacturing a wood filler and primer consisting, 1st,—in boiling a quantity of raw linseed oil for about 4 hours; 2nd,—adding a quantity of litharge and thoroughly mixing the same with the oil thus boiled; 3rd,—continue boiling the oil for another hour, add and thoroughly mix a quantity of sugar of lead; 4th,—continue boiling the compound for an additional four or five 85 hours or until the same is reduced to about the consistency of thick honey; 5th,—remove from the fire and add benzin until the compound is dissolved and liquefied to the consistency of varnish; 6th,—add and thoroughly mix a quantity of talc, all compounded and mixed in substantially the proportions above set forth.

In testimony whereof I affix my signature in the presence of two witnesses.

JOHN B. E. VENNER.

Witnesses:

JAS. B. ERWIN,

O. R. ERWIN.